

## UNITED STATES PATENT OFFICE.

GEORGIA CODDINGTON TAYLOR, OF CHARLOTTE, NORTH CAROLINA.

## COATING COMPOSITION.

No Drawing.

Application filed April 14, 1922. Serial No. 552,784.

*To all whom it may concern:*

Be it known that I, GEORGIA C. TAYLOR, a citizen of the United States, residing at Charlotte, in the county of Mecklenburg and 5 State of North Carolina, have invented certain new and useful Improvements in Coating Compositions; and I do hereby declare the following to be a full, clear, and exact description of the invention, such as 10 will enable others skilled in the art to which it appertains to make and use the same.

This invention relates to a new and useful composition of matter which is designed to be applied to fabrics, especially wearing 15 material for increasing the wearing qualities thereof. The composition is intended to be applied to the garment or fabric at the points of greatest wear by rubbing the composition into the fabric.

20 The composition consists of the following ingredients in substantially the proportions specified below:

1 pound of paraffin, 1 ounce boric acid,  $\frac{4}{10}$  grains cocoanut oil (troy weight).

25 If desired, suitable coloring matter and perfume may be added to the above ingredients to give the product a pleasing appearance and pleasant odor. I have found that one grain of pure coloring matter, preferably pink, gives the product a pleasing 30 appearance and about one grain of perfume gives the same a pleasing odor.

The composition is compounded by first 35 heating the paraffin nearly to boiling point, preferably in a double boiler, and then pouring it over the boric acid and there- after stirring the mixture to obtain thor- ough mixture of the ingredients. After thorough mixing has been obtained and as

much as possible of the boric acid has been 40 dissolved in the paraffin, the cocoanut oil is next stirred in and the coloring material and the perfume may thereafter be added.

The composition is applied to the fabric such as stockings, either before or after 45 inserting the foot, by thoroughly and vig- orously rubbing it into the fabric at the points most likely to be worn through such as the toe, heel, knee or where garters are attached. The composition, due to the par- 50 affin, serves to reduce the friction between the fabric and the parts rubbing thereon, such as the shoe or toes, and consequently increases the length of life of the garment or fabric. The composition is primarily 55 designed to be used on stockings to prevent the toes from wearing holes in the same, but may be used wherever desirable.

The ingredients comprising the compo- 60 sition are inexpensive and the composition is soothing and comforting to the feet of the user. It is perfectly harmless and will therefore, not have any injurious effects on the tenderest skin.

What I claim is:

1. A coating composition consisting of 65 paraffin, boric acid and cocoanut oil.

2. A coating composition consisting of one pound of paraffin, one ounce of boric acid, and four-tenths grains of cocoanut 70 oil.

3. A coating composition consisting of paraffin, boric acid, cocoanut oil, perfume, and coloring matter.

In testimony whereof I affix my signa- 75 ture.

GEORGIA CODDINGTON TAYLOR.